



US005977698A

# United States Patent [19]

Lee

[11] Patent Number: 5,977,698

[45] Date of Patent: Nov. 2, 1999

[54] **COLD-CATHODE EMITTER AND METHOD FOR FORMING THE SAME**

[75] Inventor: John K. Lee, Meridian, Id.

[73] Assignee: Micron Technology, Inc., Boise, Id.

[21] Appl. No.: 09/116,685

[22] Filed: Jul. 16, 1998

**Related U.S. Application Data**

[62] Division of application No. 08/554,551, Nov. 6, 1995.

[51] **Int. Cl.<sup>6</sup>** ..... H01J 1/30[52] **U.S. Cl.** ..... 313/336; 313/495; 313/309; 313/351; 313/496; 257/12; 257/22[58] **Field of Search** ..... 313/495, 309, 313/336, 351; 257/22, 10-12**References Cited****U.S. PATENT DOCUMENTS**

3,970,887 7/1976 Smith et al. ..... 313/309

|           |         |                     |           |
|-----------|---------|---------------------|-----------|
| 5,151,061 | 9/1992  | Sandhu .....        | 445/24    |
| 5,186,670 | 2/1993  | Doan et al. .....   | 445/24    |
| 5,229,331 | 7/1993  | Doan et al. .....   | 437/228   |
| 5,359,256 | 10/1994 | Gray .....          | 313/169   |
| 5,391,259 | 2/1995  | Cathey et al. ..... | 156/643   |
| 5,572,041 | 11/1996 | Betsui et al. ..... | 257/10    |
| 5,605,215 | 2/1997  | Jaskie et al. ..... | 313/336 X |
| 5,683,282 | 11/1997 | Liu et al. .....    | 313/336 X |

Primary Examiner—Ashok Patel  
Attorney, Agent, or Firm—Seed and Berry LLP

[57]

**ABSTRACT**

A cold-cathode emitter includes a high-voltage tank of a second conductivity that is formed in a substrate having a first conductivity. An emitter tip is integral with the tank and extends outwardly from the substrate. The tank forms either a drain region or a collector region of a transistor. A cold-cathode emitter device includes a drive transistor formed in a substrate of a first conductivity. The transistor includes an electron receive region of a second conductivity. An emitter tip is integral with the electron receive region and extends outwardly from the substrate.

**12 Claims, 3 Drawing Sheets**



*Fig. 1*



*Fig. 2*



*Fig. 3*



Fig. 4



Fig. 5



Fig. 6



Fig. 7



Fig. 8

## COLD-CATHODE Emitter AND METHOD FOR FORMING THE SAME

### CROSS-REFERENCE TO RELATED APPLICATION

This application is a divisional of U.S. patent application Ser. No. 08/554,551, filed Nov. 6, 1995.

### TECHNICAL FIELD

The present invention relates generally to semiconductor devices and, more specifically, to a cold-cathode device for emitting electrons in a field emission display and a method for forming the cold-cathode device.

### BACKGROUND OF THE INVENTION

A field emission display (FED) is a type of flat panel display that engineers have developed to replace the cathode ray tube (CRT) display. Typically, an FED includes a plurality of cathode emitter tips that can emit electrons while "cold," i.e., not heated like the cathode coil of a CRT. These electrons collide with a cathodoluminescent material that coats the inner surface of a display screen. The electrons from each tip collide with the screen at a corresponding location or point. Each collision point forms all or part of a picture element, i.e., pixel, of a displayed image. The greater the collision rate at a particular pixel, the brighter the pixel appears. Likewise, the lower the collision rate, the dimmer the pixel appears. A screen that displays the image in color typically includes one pixel for each component color.

An active matrix FED, which has been described in the literature, includes a drive transistor that is formed as part of the FED. Thus, the active matrix provides faster pixel signal response times and more precise brightness and color control as opposed to passive matrix FEDs, which are driven by off-FED drive transistors.

Each cathode emitter tip of an active matrix FED is typically coupled to the electron receiving region of a drive transistor. That is, the tip is coupled to either the drain of a field effect transistor or the collector of a bipolar transistor. Often, the tip is formed directly on the electron receiving region. When the transistor is activated, i.e., turned on, electrons flow through the transistor and out of the tip toward the display screen. The greater the electron flow, i.e., current, through the tip, the greater the electron collision rate at the pixel associated with the tip, and thus the brighter the pixel.

Because it is physically disposed between the drive transistor and the display screen, the emitter tip typically is formed after the drive transistor. Forming the tip after forming the drive transistor may increase the complexity of the FED manufacturing process. Furthermore, the coupling between the tip and the electron receiving region of the drive transistor may weaken over time, and thus reduce the lifetime of the tip, i.e., the time during which the tip can effectively emit electrons.

### SUMMARY OF THE INVENTION

In accordance with one aspect of the present invention, a cold-cathode emitter is provided. The cold-cathode emitter includes a high-voltage tank of a second conductivity that is formed in a substrate having a first conductivity. An emitter tip is integral with the tank and extends outwardly from the substrate. In a related aspect of the invention, the tip has a conical shape. In another related aspect of the invention, the tank forms either a drain region or a collector region of a transistor.

In accordance with another aspect of the present invention, a cold-cathode emitter device is provided. The device includes a drive transistor formed in a substrate of a first conductivity. The transistor includes an electron receive region of a second conductivity. An emitter tip is integral with the electron receive region and extends outwardly from the substrate. In a related aspect of the invention, the electron receive region forms a high-voltage tank. In another related aspect of the invention, the tip has a conical shape. 5 In yet another related aspect of the invention, the transistor includes a source and a channel that is interposed between the electron receive region, which forms a drain of the transistor, and the source. Or, the transistor includes a transistor emitter and a transistor base that is interposed 10 between the electron receive region, which forms a collector of the transistor, and the transistor emitter. 15

An advantage of the present invention is that the drive transistor and the emitter tip may be formed during the same process. Another advantage of the invention is that the emitter tip is integral with the electron receiving region of the drive transistor.

Still another advantage of the invention is that it takes advantage of the active matrix scheme, which provides a faster signal response at the emitter

### BRIEF DESCRIPTION OF THE DRAWINGS

FIG. 1 is a cross section of a portion of a field emission display (FED) according to the present invention.

FIG. 2 is a cross-sectional view illustrating the emitter structure of FIG. 1 before the formation of the emitter tip.

FIG. 3 illustrates the emitter structure of FIG. 2 after the formation of the emitter tip.

FIG. 4 illustrates the emitter structure of FIG. 3 after the formation of the field oxide, gate insulator, and gate.

FIG. 5 illustrates the emitter structure of FIG. 4 after the formation of the multi-level insulator and grid layers, and the chemical mechanical planarization of the grid layer.

FIG. 6 illustrates the emitter structure of FIG. 5 after the formation of a grid insulating layer, the emitter cavity, and the contact openings.

FIG. 7 is a circuit diagram of a cold-cathode select and drive circuit according to the present invention.

FIG. 8 is a video receiver and display device that incorporates the present invention.

### DETAILED DESCRIPTION OF THE INVENTION

FIG. 1 is a cross-sectional view of a field emission display (FED) 10 formed in accordance with the present invention. The FED 10 includes a p-type silicon substrate 12. An electron emitter 14, which includes a base 16 and one or more tips 18, is formed in the substrate 12. Multiple tips 18 are typically provided to insure a pixel will be functional if one or more of the tips 18 are defective. Because the total electron flow per pixel is maintained at a substantially constant level, a change in the number of associated tips 18 has little or no effect on the brightness of the pixel. For clarity, only one tip 18 per pixel is discussed below. Typically, the base 16 forms the electron receiving region of a drive transistor such as transistor 58 (FIG. 6). In one aspect of the invention, the base 16 is a high-voltage n tank that forms the drain of the high-voltage emitter-tip drive transistor 58, which includes a gate insulator 50, a gate 52, a channel region 59, and a source 56 (FIG. 5). The tips 18 are sometimes referred to as a conical micro-cathode.

As shown, the tip 18 of the FED 10 is surrounded by a cavity 20, which is formed in an insulator 22 and an overlying grid 24. A display screen 30 includes a glass layer 32 having on its inner surface a transparent and conductive Indium Tin Oxide (ITO) layer or anode 34, and a coating 36 of one or more phosphors. A voltage source 38 biases the grid 24 at a first positive voltage with respect to the substrate 12 biases the anode 34 at a second positive voltage that is higher than the first positive voltage applied to the grid 24. In one aspect of the invention, the grid 24 is biased to 30–110 volts and the anode 34 is biased to 1 kv–2 kv volts with respect to the substrate 12.

As shown, the emitter tip 18 is formed from the same material as and is thus integral with the base 16. Such a structure reduces the complexity of the FED 10 formation process, and increases the lifetime of the tip 18 because there is no intermediate coupling medium required between the tip 18 and the base 16.

In operation, the drive transistor 58 turns on to allow a current to flow from the tip 18 through the base 16 to the source 56. As this current flows, electrons are emitted from the tip 18. The voltage applied to the anode 34 accelerates these electrons towards the phosphors 36. As the electrons strike the atoms of the phosphors, these atoms emit light to form all or part of a pixel of the image that is displayed on the screen 30. For a color screen 30, the phosphors 36 are typically arranged to emit the appropriate combinations of colored light so as to create a color display image. For example, in one aspect of the invention, each pixel is designated either red, green, or blue.

The structure and operation of FEDs are further discussed in U.S.

Pat. No. 5,186,670, which issued to Doan et al. on Feb. 16, 1993 and is incorporated by reference herein.

Referring to FIGS. 2–6, a method is described for forming the electron emitter 14 and the associated structures of the FED 10. Referring to FIG. 2, the base 16, which in this embodiment is a high-voltage n tank, is formed in the p-type substrate 12. In one aspect of the invention, using photolithography, a photo-pattern (not shown) is formed over the substrate 12. Phosphorus is then implanted through the mask pattern at a dosage of approximately  $2 \times 10^{12}/\text{cm}^2$ – $5 \times 10^{12}/\text{cm}^2$ . The phosphorous is then further driven into the substrate 12 for approximately 5 to 7 hours at a temperature of approximately 1100° C. to 1150° C. to form the tank 16. A layer of silicon dioxide 40 is formed over the substrate 12 as a byproduct of the drive-in step. Because the base 16 is a high voltage tank region, the tank/substrate junction can withstand the voltages imparted to the grid 24 without breaking down.

Referring to FIG. 3, a tip mask (not shown) is then formed over the n tank 16. The unmasked areas of the oxide layer 40, the substrate 12, and the n tank 16 are then etched to form the tip 18. In one aspect of the invention, a plasma source dry etch that combines isotropic and anisotropic etching techniques is used to form the tip 18. Wet etching may be used as well. For a dry etch process, a fluorine base plasma source may be used. Furthermore, the base plasma may be combined with chlorine chemistry to optimize the etching ratio in a conventional manner.

Still referring to FIG. 3, a pad oxide layer 42 and a nitride layer 44 are formed over the substrate 12, the base 16, and the tip 18. The nitride layer 44 is then etched such that after the etching, the layers 42 and 44 approximately cover only the areas that will become the active areas of the FED 10.

Referring to FIG. 4, using the well-known LOCOS process, field oxide 46 is then grown in the areas of the

substrate 12 and the n tank 16 in which the nitride layer 44 has been removed. A photoresist mask (not shown) is formed over the active areas, and boron is implanted through the field oxide 46 to form p-type isolation regions 48. In one aspect of the invention, the boron is implanted at a dosage of approximately  $1 \times 10^{14}/\text{cm}^2$ – $1 \times 10^{15}/\text{cm}^2$ . In another aspect of the invention, the isolation regions 48 may be formed before the field oxide 46 is formed.

Still referring to FIG. 4, after the isolation photoresist mask is stripped, the nitride layer at 44 and the pad oxide layer 42 are removed from the active areas. Next, the gate insulator 50, which in one embodiment of the invention is formed from silicon dioxide, is formed as shown. A polysilicon gate 52 is then formed on the gate insulator 50. The tip 18 and the gate 52 are then doped n+. This doping forms a layer 54 along the outer surfaces of the tip 18. During this implantation step, the source 56 of the high-voltage drive transistor 58 is also formed. Also formed during this step are the source and drain of the low-voltage selection transistor 72 (FIG. 7), which is serially coupled to the source 56 of the high-voltage drive transistor 58. In one aspect of the invention, arsenic or phosphorous is implanted at a dosage of approximately  $6 \times 10^{15}/\text{cm}^2$ – $9.9 \times 10^{15}/\text{cm}^2$  to dope gate 52 and to form layer 54, source 56, and the sources and drains of the low voltage selection transistors 72. The dopant is then driven in using any of a number of well-known steps. In one aspect of the invention, the arsenic is driven in for  $\frac{1}{2}$  hour at approximately 900° C.–950° C. As a result of this doping, a channel 59 is formed between the source 56 and the tank 16.

Referring to FIG. 5, the insulator 22 is then formed on the exposed portions of the substrate 12, gate 52, source 56, tip 18, and field oxide 46. In one aspect of the invention, the insulator layer 22 is a deposited  $\text{SiO}_2$  layer. In another aspect of the invention, the insulator layer 22 may include multiple layers of different insulator materials, such as boron phosphate silicon glass (BPSG).

Still referring to FIG. 5, the electrically conductive grid layer 24 is then formed on the layer 22. In one aspect of the invention, the grid layer 24 is formed from polysilicon. The grid layer 24 is then subjected to chemical mechanical planarization (CMP) to expose a portion of the insulator layer 22 that is aligned with the tip 18. Next, the grid layer 24 is doped. In one embodiment of the invention, the polysilicon grid layer 24 is implanted with phosphorous at a dosage of approximately  $6 \times 10^{15}/\text{cm}^2$ – $9.9 \times 10^{15}/\text{cm}^2$ . This dopant is then driven in for approximately 10–20 minutes at a temperature of approximately 850° C.–900° C.

Referring to FIG. 6, the grid layer 24 is photoetched to form the grid 24. A second insulating layer 64 is then formed on the exposed portions of the grid 24 and the first insulating layer 22. The layer 64 may have a multilevel oxide structure, or may have another suitable structure. Contact openings 66 and 68 are then formed in alignment with the source 56 and the gate 52. Metal interconnection lines (not shown) are then formed to couple the source 56 and the gate 52 to the appropriate control lines. A passivating layer (not shown) may then be deposited on the wafer structure.

Still referring to FIG. 6, a photoresist is formed, and a buffered hydrofluoride (HF) wet etch is then used to form the cavity 20, which exposes the tip 18 and the inner surfaces of the grid 24, layer 22, and layer 64 that form the cavity 20. The remaining photoresist (not shown) is then stripped away and the bond pads are opened.

FIG. 7 is a schematic diagram of a cold-cathode select and drive circuit 70 according to the present invention. As

shown, circuit 70 includes the high-voltage drive transistor 58, which has its drain D coupled to the tip 18, its gate G coupled to a row line, its substrate biased to ground, and a source S. The circuit 70 also includes the low voltage transistor 72, which has its drain D coupled to the source S of transistor 58, its gate G coupled to a column line, its substrate biased at ground, and a source S. In another aspect of the invention, the substrate is biased at a negative voltage. The circuit 70 also includes a current limiting impedance 74, such as a current limiting resistor, which is coupled between 10 the source S of the transistor 72 and ground.

In operation, each tip 18 is located at the intersection of a particular row and a particular column. When both the row and column are selected, the tip 18 is activated. A voltage level on the row and the column line that is sufficient to turn 15 on transistors 58 and 72, respectively, serves as a select signal. Thus, when both the row line and column line that are coupled to circuit 70 carry a select signal, both the transistors 58 and 72 are activated. The simultaneous activation of both transistors 58 and 72 allows a current to flow from the 20 tip 18 through the transistors 58 and 72 and the impedance 74 to ground. The impedance 74 limits the current flowing through the tip 18 to a predetermined maximum value determined by the column signal coupled to the gate of the 25 transistor 72.

FIG. 8 is a block diagram of a video receiver and display 30 76 that incorporates the present invention. Circuit 76 includes a conventional tuner 78 that receives one or more broadcast video signals from a conventional signal source such as an antenna 80. An operator (not shown) programs, or otherwise controls, the tuner 78 to select one of these broadcast signals and to output it as a video signal. The tuner 78 may generate the video signal at the same carrier frequency as the selected broadcast signal, at a baseband 35 frequency, or at an intermediate frequency, depending upon the design of the circuit 76.

The tuner 78 couples the video signal to a conventional video processor 82 and a conventional sound processor 84. The sound processor 84 decodes the sound component of the 40 video signal and provides this sound signal to a speaker 86, which converts the sound signal into audible tones. The video processor 82 decodes, or otherwise processes, the video component of the video signal and generates a display signal. The video processor 82 may generate the display signal as either a digital or an analog signal, depending upon the design of the circuit 76. The video processor 82 couples the display signal to the FED 10, which converts the display signal into a visible image.

In one aspect of the invention, the sound processor 84 and the speaker 86 are omitted such that the circuit 76 provides only a video image. Furthermore, although shown coupled to the antenna 80, the tuner 78 may receive broadcast signals from other conventional sources, such as a cable system, a satellite system, or a video cassette recorder (VCR). Alternatively, the tuner 78 may receive a non-broadcast video signal, such as from a closed circuit video system. In such a case where only one video signal is input to the circuit 76, the tuner 78 may be omitted and the video signal may be directly coupled to the inputs of the video processor 82 and 55 the sound processor 84.

It will be appreciated that, although specific embodiments of the invention have been described herein for purposes of illustration, various modifications may be made without departing from the spirit and scope of the invention. 60 Accordingly, the invention is not limited except as by the appended claims. For example, the high voltage n tank 16

may be formed after either or both the tip 18 and the field oxide 46. Additionally, although described as having field effect transistors, the FED 10 may incorporate bipolar transistors, where the high-voltage tank 16 forms the collector of the drive transistor 58.

I claim:

1. A device for displaying a video image, comprising: a video processing circuit operable to receive and process a video signal, and to generate a display signal from said video signal; and a field emission display operable to receive said display signal and to generate said video image from said display signal, said field emission display including: a display screen having an inner surface; a cathodoluminescent coating disposed on said inner surface; a grid disposed a predetermined distance from said inner surface, said grid defining a first plurality of openings; and a plurality of cold-cathode emitters each including: a substrate having a surface and a first conductivity; an electron receiver formed in said substrate and having a second conductivity type opposite the first conductivity type; an electron supplier formed in said substrate and having said second conductivity type; a tip formed integrally with said electron receiver, extending beyond said surface in alignment with said openings, and having said second conductivity, said tip operable to emit electrons through said opening toward said inner surface; a control region formed in said substrate between said electron receiver and said electron supplier; gate oxide overlying each of said control region, a portion of said electron receiver, and a portion of said electron supplier; and a gate formed on said gate oxide, said gate overlapping a portion of said electron receiver and a portion of said electron supplier.

2. The device of claim 1 wherein said display further comprising a grid insulator that defines a second plurality of openings aligned with said first plurality of openings and is interposed between said substrate and said grid.

3. The device of claim 1 wherein said electron receiver forms a high-voltage, donor-type tank.

4. The device of claim 1 wherein said display further comprises a focus plate that is disposed between said grid and said inner surface and has a second plurality of openings that are aligned with said first plurality of openings.

5. The device of claim 1, further comprising a tuner operable to receive a plurality of broadcast signals, select one of said broadcast signals, and provide said selected broadcast signal as said video signal.

6. The device of claim 1, further comprising:

a field oxide positioned between respective portions of said gate and said electron receiver, where at least one portion of said gate extends over said field oxide.

7. The device of claim 1, further comprising:

a field oxide positioned between respective portions of said gate and said electron receiver, where at least one portion of said electron receiver extends beyond said field oxide to contact a portion of said gate oxide.

8. The device of claim 1, further comprising:

a field oxide positioned between respective portions of said gate and said electron receiver, where at least one portion of said gate extends over said field oxide and at

least one portion of said electron receiver extends beyond said field oxide to contact a portion of said gate oxide.

9. A cold-cathode emission display device, comprising:  
 a video processing circuit operable to receive and process 5  
 a video signal and to generate a display signal from said  
 video signal; and  
 a field emission display operable to receive said display  
 signal and to generate a video image from said display 10  
 signal, said field emission display including:  
 a display screen having a cathodoluminescent coating  
 disposed on an inner surface thereof;  
 an extraction grid spaced from said display screen, said 15  
 extraction grid defining at least one opening; and  
 a cold-cathode emitter formed on a substrate having a  
 surface and a first conductivity type, the cold-  
 cathode emitter including:  
 an electron supplier formed in said substrate and 20  
 having a second conductivity type;  
 an electron receiver formed in said substrate and  
 having said second conductivity type;  
 a tip formed integrally with said electron receiver,  
 extending beyond said surface and aligned with 25  
 said opening in said extraction grid, and having  
 said second conductivity type;  
 a control region formed in said substrate between  
 said receiver and said supplier;

a gate oxide overlying each of said control region, a portion of said electron receiver, and a portion of said electron supplier; and

a gate formed on said gate oxide, said gate overlapping a portion of said electron receiver and a portion of said electron supplier; and  
 a field oxide formed adjacent said tip, said gate, said gate oxide and said electron receiver, a portion of said electron receiver contacting a portion of said gate oxide, a portion of said gate extending over said field oxide.

10. The display device of claim 9, further comprising:  
 a grid insulator disposed on said substrate; and  
 a grid conductor disposed on said grid insulator such that  
 said grid insulator and said grid conductor together  
 form a cavity around a portion of said tip.

11. The device of claim 9 wherein:  
 said first conductivity type is acceptor type; and  
 said second conductivity type is donor type.

12. The device of claim 9 wherein:  
 said electron supplier forms a transistor source;  
 said electron receiver forms a transistor drain; and  
 said control region forms a transistor channel containing  
 the switching action of an electron flow from electron  
 supplier to electron receiver.

\* \* \* \* \*

UNITED STATES PATENT AND TRADEMARK OFFICE  
**CERTIFICATE OF CORRECTION**

PATENT NO. : 5,977,698  
DATED : November 2, 1999  
INVENTOR(S) : John K. Lee

Page 1 of 1

It is certified that error appears in the above-identified patent and that said Letters Patent is hereby corrected as shown below:

Column 6.

Line 21, reads "and a first conductivity;" should read -- and a first conductivity type; --

Signed and Sealed this

Twenty-eighth Day of August, 2001

*Attest:*

*Nicholas P. Godici*

*Attesting Officer*

NICHOLAS P. GODICI  
*Acting Director of the United States Patent and Trademark Office*